

## UNITED STATES PATENT OFFICE

2,382,188

## OXIDATION OF VAT AND SULPHUR DYES

George P. Vincent, Briarcliff Manor, N. Y., and Archie L. Dubéau, Rumford, R. I., assignors to The Mathieson Alkali Works, Inc., New York, N. Y., a corporation of Virginia

No Drawing. Application February 4, 1943,  
Serial No. 474,716

10 Claims. (Cl. 8—34)

This invention relates to the dyeing of textile materials. It relates more particularly to improvements in the after-treatment following the impregnation of the textile material with the dyestuff.

The invention is applicable generally to the treatment of cellulosic textiles, comprising either natural or artificial cellulosic fibers such as cotton, linen and regenerated cellulose, in the dyeing thereof with dyes, such as the so-called vat dyes and sulphur dyes, which require an after-treatment with an oxidizing agent to bring out the color or improve the fastness thereof, or both.

The vat dyes, for instance, are normally highly insoluble in water and in their use they must first be converted to a water-soluble form. The solubilization of these dyes is usually effected by the use of a reducing agent such as hydrosulphite in an alkali solution. The textile material to be dyed is impregnated with the solution of the reduced dye, generally designated a leuco solution, and must thereafter be subjected to an oxidation to restore the dye, with which the textile has been impregnated, to the insoluble form.

The reduced or leuco solution of many vat dyes has a color distinctly different from the unreduced dye, and the normal color is restored by the oxidation. This oxidation of these vat dyes is ordinarily effected by treating the impregnated textile with an aqueous solution of sodium dichromate and acetic acid.

While generally satisfactory results have been obtained by such oxidation treatment, the use of sodium dichromate and acid for this purpose has several disadvantages. In the first place, for an adequate supply of dichromate, we are dependent upon importation from distant war zones. Also, where dichromate is used, the oxidation treatment must be followed by a very thorough washing to avoid deleteriously affecting the shade of the dyed textile and prevent "skin rash." The dichromate has a tendency to dull the shade of the textile and, if the oxidation temperature is permitted to go too high, an insoluble chromium compound is formed in the cloth which cannot be washed out. Further, the use of dichromate and acid constitutes a nuisance and a hazard around the plant.

Our present invention contemplates an improved method of effecting the oxidation of the dyestuff whereby the use of chromium compounds and its attendant disadvantages are avoided. In accordance with one aspect of our invention,

the use of acid in the oxidation treatment may also be avoided.

We have found that the oxidation of the dyestuff may with advantage be effected by treatment with sodium chlorite. The chlorite may be used in conjunction with an acid, for instance the acetic acid conventionally employed. However, we have found that the use of both dichromate and acid may with advantage be avoided by using as the oxidation bath an aqueous solution of sodium chlorite and a buffer salt such as sodium bicarbonate.

The reduced dyestuff may be oxidized on the fabric in accordance with our invention by the use of the chlorite alone. However, we have found that, where the pH of the textile is reduced by the use of an acid or sodium bicarbonate or the like in conjunction with the chlorite, the oxidation proceeds more rapidly. Various acid salts or buffer salts such as phosphates may be used for the purpose of lowering the pH but we have obtained particularly satisfactory results by using sodium bicarbonate in conjunction with the chlorite, as hereinafter more fully described.

The invention is also applicable to the after-treatment of textile materials which have been dyed with a so-called sulphur dye. Some of the sulphur dyes appear to be directly soluble in water. However, for dissolving others, solubilizing agents such as sodium sulphide and sodium carbonate are customarily used. Though sulphur dyes may sometimes be used with no subsequent oxidation treatment, the textile impregnated therewith is usually treated with an aqueous oxidizing solution such as a solution of sodium dichromate and acetic acid, similar to the oxidizing treatment of vat dyes described above, in order to produce heavier shades and to improve the fastness of the dyed textile, especially its fastness to washing.

In general, our improved method of oxidizing vat dyes with which the textile is impregnated and the after-treatment of textiles dyed with sulphur dyes is substantially the same, except that in the latter a slightly lower temperature is usually employed. It comprises treating the textile, while impregnated with the dyestuff, and which may have been subjected to preliminary washing, with an aqueous solution of sodium chlorite advantageously containing also sodium bicarbonate. In place of sodium bicarbonate, a weak acid such as acetic acid or a phosphate buffer salt may be used as previously noted. The chlorite

solution may also with advantage contain a detergent such as tetrasodium pyrophosphate.

The concentration of the chlorite in the solution is not critical with respect to injury to the textile fibers and may be varied over a considerable range without harmful results. Generally at higher concentrations the oxidation proceeds more rapidly. Chlorite is consumed by the oxidation treatment. Therefore, either sufficient chlorite to complete the oxidation should be originally added or additional chlorite added as the oxidation proceeds. The optimum concentration of chlorite to be used in any particular operation will vary somewhat, depending upon special conditions but is readily determinable in the light of the present disclosure.

The dye-impregnated textile is ordinarily highly alkaline as it comes from the dye bath. As previously noted, we have found the chlorite oxidation of the dye to proceed more rapidly and to be generally more satisfactory, if the composition of the chlorite solution be such as to reduce the alkalinity of the impregnated textile. Particularly satisfactory results are usually obtained by maintaining the alkalinity of the bath within the range of about pH 8 to about pH 10.5. However, a pH from about 3 up to that approximating the pH of caustic soda may be used. Though the oxidation of the dyestuff may be effected by the chlorite in an acid solution this is not usually as desirable as a somewhat alkaline solution because of a tendency toward excessive generation of gases and danger of corrosion.

The reduction of alkalinity is advantageously effected, in accordance with our invention, by the inclusion in the chlorite solution of an amount of an alkalinity reducing substance adequate to produce the desired pH reduction. Sodium bicarbonate has been found particularly satisfactory for this purpose. Because of the characteristic pH of sodium bicarbonate, the alkalinity of the oxidizing solution is thereby readily maintained at an optimum pH value of about 8.3 or within the range of about pH 8 to about pH 10, and extra care to avoid using excessive quantities of the acidic constituent is unnecessary.

An oxidizing solution which we have found generally satisfactory for the after-treatment of either vat or sulphur dyes may be prepared by dissolving about 1 pound of sodium chlorite and about 5 pounds of sodium bicarbonate in about 40 to 50 gallons of water.

A generally satisfactory oxidizing bath in which an acid is used in place of the bicarbonate may be prepared from the following ingredients and approximate proportions thereof:

Water ..... gallons 250  
Sodium chlorite ..... pounds 2  
Acetic acid (28%) ..... do 10

Advantageously, about 3 ounces of tetrasodium pyrophosphate or a similar detergent material may also be added.

In the after-treatment of the vat dyes the temperature of the oxidation bath is advantageously maintained at about 140° F. In the after-treatment of sulphur dyes it is usually desirable to maintain the bath at about 10 degrees lower temperature. In either case, somewhat higher or lower temperatures may be used.

The treatment of the textile with the chlorite solution may be effected in the manner and by the apparatus ordinarily used in conventional practice. For instance, the textile may be passed through the chlorite oxidizing bath by means of

conventional jigs. Usually the textile is passed from one roller through the bath onto a second roller. This operation may be repeated a number of times and each passage of the textile through the bath is designated an "end." Prior to and following the chlorite treatment, the textile may be given several "ends" through wash water.

Advantageously, where sodium bicarbonate is used in conjunction with the sodium chlorite, half of the chlorite and all of the bicarbonate are dissolved in the bath. The textile is given one end through this bath and then the remainder of the chlorite added and the cloth given several additional ends through the bath.

The invention will be further described by means of the following specific illustrations of its application:

#### Example I

In the vat dyeing of a 1.69 yards per pound twill an olive drab shade, using a machine jig, the fabric after having the dye padded thereon, in the conventional manner, was given three ends in a bath of hydrosulphite and caustic soda and then transferred without washing to a second jig containing 50 gallons of water to which had been added one pound of sodium chlorite dissolved in a half gallon of water, the temperature of the solution raised to 140° F., and 1½ gallons of 28% acetic acid added. The cloth was given three ends through this solution, each end requiring seven minutes, and was then washed and sent to the soaper. The available chlorine and pH of the solution during the various stages of the operation were as follows:

| Stage                 | Available Cl <sub>2</sub> | pH  |
|-----------------------|---------------------------|-----|
| Start.....            | Percent                   |     |
| After first end.....  | 0.28                      | 4.3 |
| After second end..... | 0.196                     | 4.3 |
| After third end.....  | 0.045                     | 4.3 |
|                       | 0.045                     | 4.3 |

A complete oxidation of the dye was effected by this treatment.

#### Example II

In the vat dyeing to an olive drab shade of 1.75 yards per pound poplin, the cloth was padded with the vat dye in the conventional manner and given three ends in the ordinary hydrosulphite-caustic soda solution. The cloth impregnated with the leuco solution was then washed by giving it two runs through cold water. The water bath was then dropped to fifty gallons, one pound of sodium chlorite and two quarts of 56% acetic acid added and the cloth given four ends through this oxidizing solution at a temperature of 140° F., after which it was washed by four ends through cold water followed by two ends through hot water and passed to an ordinary soap solution containing one pound of soda ash.

The condition of the oxidizing bath during the operation was as follows:

| Stage                       | Available Cl <sub>2</sub> | pH  |
|-----------------------------|---------------------------|-----|
| Beginning first end.....    | Percent                   |     |
| Middle first end.....       | 0.280                     | 4.4 |
| Beginning second end.....   | 0.177                     | 3.8 |
| Beginning third end.....    | 0.112                     | 4.2 |
| Beginning fourth end.....   | 0.074                     | 4.7 |
| Termination fourth end..... | 0.060                     | 4.7 |
|                             | 0.050                     | 4.8 |

*Example III*

In two additional runs, using an oxidation bath identical with that described in Example II, the cloth was given three ends through the chlorite bath instead of four, as in the preceding example. In the first of these runs, the cloth was given a cold water wash before "soaping down." In the second of these runs, the cloth was "soaped down" directly after leaving the oxidizing bath with an ordinary soap solution to which two pounds of soda ash had been added. In these two additional runs, and in the run described as Example II, the shade of the cloth was identical with that resulting from the dichromate oxidation ordinarily used.

From the runs of Examples II and III, it appears that, in accordance with our improved process wherein the oxidation is effected by the use of sodium chlorite, the washing operation may be materially simplified. The washing operation following the oxidation may with advantage be accomplished by subjecting the cloth immediately after the oxidation treatment to one end in cold water containing two pounds of soda ash, adding soap or a synthetic detergent directly to the soda ash solution before beginning the next end and following this, without further washing, by the ordinary "soaping down" operation.

*Example IV*

A herringbone poplin of 1.60 yards per pound was padded with an O. D. vat dye and given eight ends through the conventional hydrosulphite-caustic soda solution. Thereafter, the cloth was washed by two ends through cold running water and then subjected to oxidation and further washing. Using the conventional oxidation bath prepared from two pounds of sodium dichromate and four quarts of 56% acetic acid, the oxidation required four ends and the subsequent washing, prior to soaping down, required four ends of the cloth through hot running water. In accordance with our improved method, by the use of an oxidation bath prepared from 1½ to 2 pounds of sodium chlorite and 2½ quarts of 56% acetic acid, complete oxidation was effected by only three ends through the bath, and the subsequent washing was effected by only one end through hot running water prior to soaping down instead of four runs required by the conventional method. In each case the temperature of the oxidation bath was maintained at 140° F. The shade of the fabric treated by our improved method was identical with that resulting from the conventional dichromate oxidation.

In the above run, only one pound of the chlorite was originally added. Half way through the first end the available chlorine had dropped to 0.08% and an additional ½ to 1 pound of the chlorite was added at the beginning of the second end. At the start of the first end, the pH of the chlorite solution was 3.5 and at the termination of the third end it was 6.

In the preceding examples, the pH of the chlorite solution was maintained on the acid side. As we have previously noted, it is frequently desirable to use an alkaline chlorite solution. This is readily accomplished by the use of sodium bicarbonate or other salts capable of regulating the pH of the solution, in conjunction with the chlorite. Examples of such use of sodium bicarbonate are as follows:

*Example V*

An approximately 600 gram package of two-ply 30's mercerized yarn was treated in an experimental drum, package machine with an aqueous solution of hydrosulphite, caustic soda and synthetic detergent. A vat dye was then added and the solution in which the package was submerged was circulated continuously for about 45 minutes. The solution was then withdrawn and a fresh solution of 68 grams of sodium bicarbonate in 6 quarts of water added. The temperature was raised to 140° F., and 3.4 grams of sodium chlorite added. After circulating this solution for 3 to 4 minutes, an additional 3.4 grams of sodium chlorite was added and the circulation continued for a total of about 15 minutes after the initial addition of the chlorite. The oxidizing solution was then withdrawn and the yarn washed twice in hot water and once in warm water at a temperature of about 100° F., containing a conventional yarn conditioner.

*Example VI*

In a commercial operation in which an oxidation bath of sodium chlorite and sodium bicarbonate was used, the process was carried out as follows, the fabric being heavy twill and herringbone of two yards per pound quality: The fabric from the dye bath was given four ends through cold water and then passed to the oxidizing bath in which a temperature of 140° F., was maintained. The cloth was first given one end through the oxidizing bath containing five pounds of sodium bicarbonate and one-quarter pound of sodium chlorite in about 25 gallons of water. An additional one-quarter pound of sodium chlorite was then added and the cloth given three more ends through the oxidizing bath. Thereafter, it was given four ends through hot water at a temperature of about 180° F., followed by four ends through a soap-sodium carbonate solution, three ends through hot water and "shelled" up through cold water. The results obtained were substantially identical with those obtained by the same treatment of the fabric in the conventional manner, using an oxidizing bath of sodium dichromate and acetic acid.

*Example VII*

In dyeing a challis type fabric of 10 yards per pound spun rayon, the cloth was padded with an admixture of Indanthrene vat dye to give a green shade and the dyestuff thereon reduced by treatment for 20 minutes with an aqueous solution of sodium hydroxide and hydrosulphite in the conventional manner. Thereafter, the fabric was given two ends through wash water and passed to an oxidizing bath consisting of an aqueous solution of sodium chlorite and sodium bicarbonate. In the oxidizing treatment, the cloth was given one end through an aqueous bath to which 5 pounds of sodium bicarbonate and ½ pound of sodium chlorite had been added. Thereafter, an additional ½ pound of sodium chlorite was added to the bath and the cloth given three more ends therethrough. During this oxidation treatment, which extended over a period of about 15 minutes, the temperature of the oxidation bath was maintained at 140° F., and the pH thereof ranged from 8.3 to 8.45. Following the oxidation treatment, the cloth was given two ends through hot water and was thereafter shelled up through cold water. The results obtained by this treatment were highly satisfactory. The final washing was more readily effected than where conventional oxidiz-

ing methods are employed and there was a substantial saving in the cost of chemicals. It is possible to effect a still greater economy in chemicals employed in the foregoing operation by reducing the amounts of chlorite and sodium bicarbonate used. The bicarbonate may be reduced by at least 50% without ill effects.

I have found, particularly where sodium bicarbonate is used in conjunction with the chlorite in my improved oxidation treatment, that material economy may be effected in the washing operations preceding and following the oxidation treatment without deleteriously affecting the finished textile. Thus, in the operation described in the preceding Example VI, the washing following the oxidation and preceding the soaper may be reduced to two ends instead of four ends or this washing step may even be entirely eliminated without harmful effect on the finished cloth.

Also, because of the relatively mild but entirely effective action of the chlorite and sodium bicarbonate constituents of my oxidation bath, the textile may be passed directly from the dye bath to the oxidation bath without the usual intermediate washing. However, where this intermediate washing is omitted, more dyestuff and caustic is carried into the oxidation bath and, accordingly, more chlorite and sodium bicarbonate should be used. For example in the operation described in Example VI, where the preliminary washing is omitted, it is desirable to increase the amount of chlorite to about 1½ pounds and the amount of sodium bicarbonate to about 15 pounds. Under similar conditions, where the preliminary washing is not wholly omitted but is reduced to two ends instead of four ends, about 1 pound of chlorite and about 12 pounds of sodium bicarbonate are usually sufficient. In either case, it is advantageous to add about one-half of the chlorite to the oxidation bath prior to the first end and the remainder following the first end.

As previously noted, the after-treatment of textiles dyed with sulphur dye, in accordance with my present invention, is substantially the same as the previously described and illustrated after-treatment of vat dyed fabrics except that a slightly lower temperature is generally desirable. My after-treatment of sulphur dyes is illustrated by the following specific examples:

#### Example VIII

A poplin of about 1.7 yards per pound, after impregnation with an admixture of sulphur dyestuff to give a brown shade, was passed without washing from the dyeing operation to a jig containing about 50 gallons of an aqueous solution to which had been added 1 pound of sodium chlorite dissolved in ½ gallon of water, the temperature of the solution raised to 130° F., and 1½ gallons of 28% acetic acid added. The cloth was given three ends through this solution and then washed and sent to the soaper. During the treatment with the chlorite solution, the temperature of the bath was maintained at 130° F. Entirely satisfactory results were obtained, the cloth being brightened and the wash-fastness of the dyed fabric substantially improved.

#### Example IX

A heavy twill of 2 yards per pound quality, which had been impregnated with a sulphur dye to give a blue-green shade, was given 4 ends in cold water and thereafter subjected to treatment in an aqueous solution of sodium chlorite and sodium bicarbonate maintained at a temperature of 130° F. This bath was prepared by adding to

about 25 gallons of water 5 pounds of sodium bicarbonate and ¼ pound of sodium chlorite. The cloth was given one end through this bath followed by three more ends through the bath after an additional ¼ pound of sodium chlorite had been added. The cloth was then given four ends through hot water and passed to the soaper.

As in the treatment of vat dyes previously discussed herein, the washing operations preceding and following the treatment with the sodium chlorite may be materially reduced from that of the preceding example, particularly where sodium bicarbonate is used in conjunction with the chlorite. Where my chlorite-bicarbonate bath is employed, the dye fabric may be passed directly to the after-treatment with no intermediate washing or it may be given only two ends through the wash water. Following the chlorite treatment, the cloth may be passed immediately to the soaper or it may be subjected to a mild washing operation, say two ends through the wash water. However, some washing prior to the chlorite treatment is usually desirable as by such washing the amounts of chlorite and sodium bicarbonate required are reduced.

Where the textile being treated is of a non-absorbent nature, it is desirable to include in the oxidation bath a penetrant to assist in the absorption of the oxidizing solution by the fabric.

We claim:

1. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite, having a pH not less than about 3, for a period of time sufficient to effect the desired oxidation.

2. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite and an acid, having a pH not less than about 3, for a period of time sufficient to effect the desired oxidation.

3. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite and acetic acid, having a pH not less than about 3, for a period of time sufficient to effect the desired oxidation.

4. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite and a buffer salt, having a pH not less than about 3, for a

period of time sufficient to effect the desired oxidation.

5. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite and sodium bicarbonate, having a pH not less than about 3, for a period of time sufficient to effect the desired oxidation.

6. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an alkaline aqueous solution of sodium chlorite for a period of time sufficient to effect the desired oxidation.

7. In the dyeing of cellulosic textile materials with a dyestuff of the class consisting of the sulphur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite for a period of time sufficient to effect the desired oxidation and maintaining the solution during the treatment at a pH within the range from about 8 to 10.5.

8. In the dyeing of cellulosic textile materials with a dyestuff of the class consisting of the sul-

phur dyes and the vat dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite for a period of time sufficient to effect the desired oxidation and maintaining the solution during the treatment at a pH within the range from about 8 to 10.5 by the presence of sodium bicarbonate.

9. In the dyeing of cellulosic textile materials with a dyestuff of the class consisting of vat dyes and sulphur dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite, having a pH within the range of about 8 to 10.5 and a temperature of about 130 to 140° F., for a period of time sufficient to effect the desired oxidation.

10. In the dyeing of cellulosic textile materials with a dyestuff of the class consisting of vat dyes and sulphur dyes which after application to the textile is subjected to an oxidation treatment to develop or improve its color and fastness, the improvement which comprises effecting the oxidation of the dyestuff by treating the textile impregnated with the dyestuff with an aqueous solution of sodium chlorite, containing about two pounds of sodium chlorite per one hundred gallons of solution, at a temperature of about 130 to 140° F., for a period of time sufficient to effect the desired oxidation and maintaining the pH of the solution within the range of about 8 to 10 by the presence of bicarbonate of soda.

GEORGE P. VINCENT.  
ARCHIE L. DUBEAU.